

Patented Mar. 29, 1927.

1,622,576

# UNITED STATES PATENT OFFICE.

JOHN N. EARLY, OF PITTSBURGH, PENNSYLVANIA.

## ALLOY.

No Drawing.

Application filed July 21, 1926. Serial No. 124,105.

This invention relates to an alloy of iron, the main constituents of which are iron, silicon, sulfur, phosphorus, manganese, carbon, and molybdenum, with or without small quantities of either nickel or chromium or both.

This alloy is characterized by having great strength and a very hard chill surface, also that the chill depth may be readily controlled by the operator, either in a sand or chill mold.

This alloy may be used for making all commercial castings requiring hardness and tensile strength, such as rolling mill guides, 15 rolling mill rolls, crusher rolls, and the like.

Heretofore, in casting iron alloys the chill depth has been uncontrollable, except by the use of chill pieces or chill molds, and even then has been more or less of an uncertain 20 matter, while the present alloy permits of positive control of the chill depth at all times.

Generically, the invention consists in an alloy containing the elements and the percentages thereof, following—

|                                  | Per cent.    |
|----------------------------------|--------------|
| Silicon                          | .75 to 1.50  |
| Sulfur                           | .05 to .35   |
| Phosphorus                       | .25 to .75   |
| 30 Manganese                     | .20 to .70   |
| Carbon                           | 2.00 to 3.75 |
| Nickel                           | .05 to .25   |
| Chromium                         | .15 to .25   |
| Molybdenum                       | .10 to .30   |
| 35 Iron sufficient to make 100%. |              |

Castings made from this alloy show remarkable results in tensile strength and in wearing quality, and in the resistance to 40 the action of heat.

The molybdenum increases the tensile strength of the alloy and the high sulfur content causes a greater amount of the carbon to become combined than would otherwise be the case. Molybdenum also raises the ratio of the elastic limit to the ultimate strength of the metal and benefits the ductility.

50 The most notable characteristic of this alloy aside from its great strength, is its ability to chill in either a sand or chill mold, and the ease with which the operator can control the depth of chill.

When rolls are formed from this alloy they 55 will outwear ordinary rolls made from alloys

ordinarily used for this purpose several times.

The depth of the chill on castings formed from this alloy is readily controlled by varying the sulfur content and by varying the heat at which the metal is poured.

The molybdenum may be added to the mix as molybdenum scrap, as ferro-molybdenum, or as calcium molybdate, and is preferably added after the other metals of the mix have melted and just long enough before tapping the heat to permit of it becoming thoroughly diffused throughout the bath.

The nickel and chromium serve to increase the tensile strength and toughness of the alloy and may be omitted for some purposes, however, when making rolling mill rolls chromium will preferably be used and in some cases nickel will also be used although the nickel is not essential.

In producing this novel alloy, the following method is carried out—

A cupola or other smelting furnace is first charged with suitable scrap, pigs, or ores, of the proper analysis to produce the proper proportion of silicon, sulfur, phosphorus, manganese, and carbon, and if chromium or nickel are to be included in the alloy, suitable pigs or scrap containing these ingredients are also added. After the mix is made up it is heated to from 2500 to 2700 degrees Fahrenheit to melt the metals. That is, the mix is raised to a heat materially above the melting temperature in order to obtain a good pouring temperature. The molybdenum is preferably added after the mix is melted down and just long enough before tapping the heat to permit it to become thoroughly diffused throughout the bath, although the molybdenum may be added at any time during the melting operation or as scrap when making up the mix if desired.

After the mix is melted it is tapped and then poured into the molds at a temperature of from 2300 degrees to 2500 degrees Fahrenheit.

The depth of chill on the finished casting is controlled primarily by the pouring temperature. That is, the hotter the pouring temperature the deeper will be the chill; also the depth of chill can be controlled somewhat by the sulfur content of the mix, that is, the greater the sulfur content the greater

2  
the chill. However, the sulfur content is known and when it is slightly higher or lower than necessary to produce the correct depth of chill, the pouring temperature may be increased or lowered accordingly to give the correct depth of chill.

While I have described certain specific combinations of elements within certain ranges, it will be understood that I do not wish to be limited thereto beyond the express limits of the appended claim which is meant to cover various modifications and equivalents as may be readily practiced by those skilled in the art to which this invention belongs.

I claim—

A ferrous metal alloy primarily suited for the making of castings having a hard chilled surface such as rolling mill rolls, and ca-

pable of forming a controllable chill in a sand mold without the use of chills, said alloy containing the following elements in substantially the following proportions—

|                                                 | Per cent.    | 25 |
|-------------------------------------------------|--------------|----|
| Silicon-----                                    | .75 to 1.50  | 25 |
| Sulfur-----                                     | .05 to .35   |    |
| Phosphorus-----                                 | .25 to .75   |    |
| Manganese-----                                  | .20 to .70   |    |
| Carbon-----                                     | 2.00 to 3.75 | 30 |
| Nickel-----                                     | .05 to .25   |    |
| Chromium-----                                   | .15 to .25   |    |
| Molybdenum-----                                 | .10 to .30   |    |
| Iron approximately sufficient to complete 100%. |              | 35 |

In testimony whereof, I have hereunto signed my name.

JOHN N. EARLY.